

March 13, 1928.

1,662,605

R. E. HALL

REINFORCED FIBROUS CONTAINER AND METHOD OF MANUFACTURE

Filed April 8, 1925

Fig. 1.



Fig. 2.



Fig. 3.

Fig. 4.



Fig. 5.

Witness:

Stephen Melora 3



## UNITED STATES PATENT OFFICE.

RICHARD E. HALL, OF OLEAN, NEW YORK, ASSIGNOR, BY MESNE ASSIGNMENTS, TO THE ARVEY MANUFACTURING CO., OF WILMINGTON, DELAWARE, A CORPORATION OF DELAWARE.

## REINFORCED FIBROUS CONTAINER AND METHOD OF MANUFACTURE.

Application filed April 8, 1925. Serial No. 21,463.

This invention relates to improvements in reenforced fibrous containers and method of manufacture, and refers more particularly to a reenforced felted fibrous container such as a pail and the like, having reenforcing elements imbedded during formation in the base and side wall to protect the annular edge of the base, as well as the base or side walls and to provide a more rigid construction.

10 The reenforcement may comprise wire mesh incorporated with the fibres during the felting and forming operation.

This application is in part a modification and in part an improvement of a co-pending application filed by me, Serial No. 744,586, filed October 20th, 1924. The process and apparatus there described, may be utilized to produce the novel product of the present invention, with such changes in the steps of 20 the process as shall be hereinafter pointed out.

In the drawings:

Fig. 1 is a side elevational view of a reenforced fibrous container with its base partially broken away, to expose one type of reenforcement.

Fig. 2 is a cross sectional view taken on line 2—2 of Fig. 1.

Fig. 3, Fig. 4 and Fig. 5 are vertical sectional views of containers having the reenforcement imbedded in different parts thereof.

Referring in detail to the drawings, 1 designates as a whole a seamless, felted fibrous container which, in the present instance, takes the form of a pail having the base 1' side wall 2 and open top. The process of making this container is clearly described in said co-pending application, and 20 may be briefly described as follows: The pulp solution is contained as a vat and a carrier having on its periphery spaced perforated forming molds intermittently rotated to successively submerge the molds in the pulp solution. Suction is applied on the 30 interior of the perforated mold subsequent to complete immersion, said suction being maintained until the form and pulp felted thereon have emerged from the pulp solution and have been pressed to remove excess water. Subsequent to pressing, the felted, pressed container is removed from the form. The container is then dried and the mold

again ready for immersion. The entire operation is controlled automatically.

The above describes the method of producing a felted fibrous container in which there is no reenforcement. To produce the reenforced container of the present invention, the same process and apparatus may be utilized, with the modifications herein-after pointed out. As shown in Figs. 1 and 2, a strip of say, one eighth to one-half inch mesh wire, from three to six inches wide and about thirty-three inches long is first formed into a hoop and placed upon the perforated forming mold above described, subsequent to the removal of the previously felted and pressed container, and before again immersing said perforated forming mold in the pulp solution. As the perforated forming mold is submerged in the pulp solution and suction is applied, the suction holds the reenforcing insert in place and the mesh is coarse enough so that a portion of the pulp passes therethrough; thus, very little of the wire insert is exposed on the inside of the finished pail.

It has been ascertained by test that the insertion of this wire reenforcement in a container loaded to its maximum will result in a stronger product, capable of withstanding abuse from rough handling. It is particularly to be noted that in any of the containers shown in the drawings, the annular edges of the base are protected. These edges of a pail are the spots exposed to most damage.

The container shown in Fig. 1 has the reenforcing metallic insert 3 protecting the annular edge, and extending inwardly into the base 1' for some distance and also projecting upwardly into the side wall 2. The container shown in Fig. 3 has a strip of wire mesh 5 extending entirely through the base 95 and terminating in short upward projections at line 4 in the shape of a basket.

The basket shaped insert designated as a whole at 5 is placed exterior of the container forming apparatus in a slightly larger basket 100 of very fine mesh, and pulp from the press felting tank is manually poured therein to a depth of say, one inch. In about thirty seconds while the container is being pressed (in the container forming apparatus) the 105 water flows away by gravity leaving about

one-fourth inch coating of pulp on the inside of the wire basket 5, which is to be used as an insert. The slightly larger basket of very fine mesh in which the wire basket 5 is placed, is necessary because if the pulp was poured into the basket 5 which is of coarse mesh without the larger basket of very fine mesh about it, the pulp would go through the coarser mesh. This double basket is then placed on the perforated mold of the apparatus and the outer basket of fine mesh is immediately removed. Immediately subsequent to the submerging of the pail form, a coating of pulp is thrown on the outside of the basket through the use of the suction as explained, completely hiding the wire from view on the inside or outside of the pail.

An additional side wall reenforcement 6 may be inserted in the pail shown in Fig. 3, when found desirable or necessary. In Fig. 4, the wire mesh 7 extends through base 1', terminating short of the side walls. The corner is protected by the side wall reenforcement 8 terminating in the extension 9 imbedded in the base. The construction shown in Fig. 5 is similar to that shown in Fig. 1, with the additional side wall reenforcement 10.

It is of course, to be understood that I do not in any way wish to limit myself to the particular styles and places of insert shown.

I claim as my invention:

1. A seamless fibrous container formed of felted, interlocked fibres, having integral base 31 and side walls, and reenforcing wire mesh imbedded in the base and side walls, said fibres passing through the spaces between the wire mesh and interlocking therewith and with each other on both sides of the wire mesh 40 to provide a compacted unitary structure.

2. A seamless fibrous container formed of felted, interlocked fibres, having integral base and side walls, and reenforcing wire mesh imbedded in the base and side walls 41 extending entirely across the corners, said fibres passing through the spaces between the wire mesh and interlocking therewith and with each other on both sides of the wire mesh 50 to provide a compacted unitary structure.

3. A seamless fibrous container formed of felted fibres interlocking with each other, having integral base and side walls and reenforcing material imbedded in the base and side walls and extending entirely across the corners, said fibres interlocking with said reenforcing material and with each other on both sides of the reenforcing material to produce a compacted unitary structure possessing the characteristics of having had the reenforcing material incorporated during felting of the fibres. 60

RICHARD E. HALL.